

United States Patent [19]  
Das et al.



US005229165A

[11] Patent Number: 5,229,165  
[45] Date of Patent: Jul. 20, 1993

[54] PLASMA SPRAYED CONTINUOUSLY  
REINFORCED ALUMINUM BASE  
COMPOSITES

[75] Inventors: **Santosh K. Das; Michael S. Zedalis**,  
both of Randolph, N.J.; **Paul S. Gilman**, Suffern, N.Y.

[73] Assignee: **Allied-Signal Inc.**, Morristownship,  
N.J.

[21] Appl. No.: 435,137

[22] Filed: Nov. 9, 1989

[51] Int. Cl.<sup>5</sup> ..... B05D 1/08

[52] U.S. Cl. ..... 427/456; 427/126.4;  
427/387; 427/397.7

[58] Field of Search ..... 427/34, 126.4, 387,  
427/397.7

[56] References Cited

U.S. PATENT DOCUMENTS

3,596,344 3/1971 Kreider ..... 29/419

|           |         |                |       |         |
|-----------|---------|----------------|-------|---------|
| 3,606,667 | 9/1971  | Kreider        | ..... | 29/423  |
| 3,615,277 | 10/1971 | Kreider        | ..... | 29/195  |
| 4,737,379 | 4/1988  | Hudgens et al. | ..... | 429/39  |
| 4,782,884 | 11/1988 | Siemers        | ..... | 164/46  |
| 4,786,566 | 11/1988 | Siemers        | ..... | 428/568 |
| 4,805,833 | 2/1989  | Siemers        | ..... | 228/190 |

Primary Examiner—Peter A. Nelson

Attorney, Agent, or Firm—Ernest D. Buff; Gerhard H. Fuchs

[57] ABSTRACT

A metal matrix composite is produced by forming a rapidly solidified aluminum base alloy into powder. The powder is plasma sprayed onto at least one substrate having thereon a fiber reinforcing material to form a plurality of preforms. Each of the preforms has a layer of the alloy deposited thereon, and the fiber reinforcing material is present in an amount ranging from about 0.1 to 75 percent by volume thereof. The preforms are bonded together to form an engineering shape.

29 Claims, 3 Drawing Sheets



Fig. 1



Fig. 2



Fig. 3



Fig. 4



Fig. 5



## PLASMA SPRAYED CONTINUOUSLY REINFORCED ALUMINUM BASE COMPOSITES

### BACKGROUND OF THE INVENTION

#### 1. Field of the Invention

This invention relates to a process for improving the mechanical properties of metals, and more particularly to a process for producing an aluminum composite having a rapidly solidified metal matrix and a continuous fiber reinforcement.

#### 2. Description of the Prior Art

An aluminum based composite generally comprises two components—an aluminum alloy matrix and a hard reinforcing second Phase. The reinforcing phase may be discontinuous, e.g., particulate, short fiber, or may be continuous in the form of a fiber or tape. The composite typically exhibits at least one characteristic reflective of each component. For example, a continuous fiber reinforced aluminum based composite should reflect the ductility and fracture toughness of the aluminum matrix as well as reflect of the elastic modulus and strength of the fiber.

Continuous fiber reinforced aluminum based composites are usually limited to ambient temperature applications because of the large mismatch in higher temperature strength between the aluminum matrix (low strength) and the continuous fiber reinforcement (high strength). Another problem with continuous fiber reinforced metal matrix composites produced by mechanically binding continuous fiber between aluminum based matrix foils is the difficulty in producing a bond between the matrix and the fiber. To produce such a bond it is often times necessary to vacuum hot press the material at temperatures higher than the incipient melting temperature of the matrix or higher than the stability of precipitate phases present in the aluminum based matrix. Still another problem with continuous fiber reinforced metal matrix composites produced by cold spraying a rapidly solidified aluminum based matrix mixed with an organic binder onto a continuous fiber preform and then burning off the organic binder is that the organic binder decomposes and forms a deleterious residue within the sprayed preform. An alternative method of fabricating the composites is by plasma spraying. Prior processes in which alloys and/or continuous fiber reinforced metal matrix composites are fabricated by means of plasma or arc spraying are disclosed in U.S. Pat. Nos. 3,596,344, 3,606,667, 3,615,277, 4,782,884, 4,786,566, and 4,805,833. However, all the previous work was done using atomized aluminum powder which did not have the metastable microstructure of rapidly solidified aluminum powder. Hence, there is a need for an invention for plasma spraying a rapidly solidified aluminum alloy matrix where rapid enough solidification of the molten powder droplets be attained to retain the microstructure of the starting rapidly solidified alloy.

### SUMMARY OF THE INVENTION

It is therefore proposed that the elevated temperature properties of the composite be improved, and that mechanical binding and cold spraying for fabrication be avoided by plasma a rapidly solidified, high temperature aluminum alloy onto continuous fiber preforms. This procedure, referred to as plasma provides for a high temperature aluminum base matrix free of organic residue and permits the continuous fiber reinforcement

to be bonded to the matrix without heating the material to a temperature above the solidus of the matrix. Moreover, this procedure allows for the deposition and retention of a rapidly solidified alloy onto a substrate and the improved ambient and elevated temperature mechanical and physical properties accorded from the resultant microstructure. The plasma sprayed monotapes may be subsequently bonded together using suitable bonding techniques, e.g., diffusion or roll bonding, forming engineering structural components.

Briefly state, the invention provides a process for producing a rapidly solidified aluminum base metal matrix composite, comprising the steps of:

(a) forming a rapidly solidified aluminum base alloy into a powder;

(b) plasma spraying said powder onto at least one substrate having thereon a fiber reinforcing material to form a plurality of preforms wherein each of said preforms has a layer of said alloy deposited thereon and said fiber reinforcing material is present in an amount ranging from about 0.1 to 75 percent by volume thereof; and

(c) bonding said preforms to form an engineering shape.

In addition, the invention provides a composite comprised of a plurality of preforms bonded to form an engineering shape, each of said preforms comprising a substrate having thereon a fiber reinforcing material upon which an aluminum base alloy layer is deposited, said alloy having been rapidly solidified formed into a powder and deposited by plasmac spraying, and said fiber reinforcing material being present in an amount ranging from about 0.1 to 75 percent by volume thereof.

The powder has a powder size less than—40 mesh (U.S. Standard Sieve size) when sprayed in a molten state onto a fiber reinforced substrate using plasma spraying techniques, forms a preform monotape. The fiber may be placed directly on a mandrel or on a suitable substrate such as a rolled foil or planar flow cast ribbon. In this manner there is provided a strong bond between the deposited matrix material and the surface of the reinforcing fibers. Moreover, the attractive microstructure and mechanical and physical properties of the rapidly solidified powder or wire are retained. This process may be repeated such that subsequent spraying is done on fibers placed on top of the sprayed monotapes, and the multilayered preforms may be fabricated. Upon completion of the plasma spraying step, the resultant fiber reinforced preforms are bonded together using suitable bonding techniques such as diffusion bonding, roll bonding and/or hot isostatic pressing, to form an engineering shape which is substantially void-free mass. This shape may be subsequently worked to increase its density and provide engineering shapes suitable for use in aerospace components such as stators, wing skins, missile fins, actuator casings, electronic housings and other elevated temperature stiffness and strength critical parts, automotive components such as

60 Piston heads, Piston liners, valve seats and stems, connecting rods, can shafts, brake shoes and liners, tank tracks, torpedo housings, radar antennae, radar dishes, space structures, sabot casings, tennis racquets, golf club shafts and the like.

### BRIEF DESCRIPTION OF THE DRAWINGS

This invention will be more fully understood and further advantages will become apparent when refer-

ence is made to the following detailed description of the preferred embodiment of the invention and the accompanying drawings in which:

FIG. 1 is a light photomicrograph of a fiber reinforced plasma sprayed monotape composed of rapidly solidified aluminum based iron, vanadium and silicon containing alloy matrix deposited on British Petroleum Sigma monofilament SiC fiber placed upon planar flow cast aluminum based iron, vanadium and silicon containing ribbon fabricated by the present invention;

FIG. 2 is a light photomicrograph of a fiber reinforced plasma sprayed monotape composed of rapidly solidified aluminum based iron, vanadium and silicon containing alloy matrix deposited on Nicalon multi-filament SiC fiber impregnated with aluminum, placed upon planar flow cast aluminum base iron, vanadium and silicon containing ribbon fabricated by the present invention;

FIG. 3 is a transmission electron photomicrograph of a deposited layer plasma composed of rapidly solidified aluminum based iron, vanadium and silicon containing alloy;

FIG. 4 is a photomicrograph of diffusion bonded layers of plasma sprayed monotapes composed of rapidly solidified aluminum based iron, vanadium and silicon containing alloy matrix deposited on British Petroleum Sigma monofilament SiC fiber placed upon planar flow cast aluminum based iron, vanadium and silicon containing ribbon fabricated by the present invention;

FIG. 5 is a photomicrograph of diffusion bonded layers of plasma sprayed monotapes composed of rapidly solidified aluminum based iron, vanadium and silicon containing alloy matrix deposited on Nicalon multi-filament SiC fiber impregnated with aluminum, respectively, placed upon planar flow cast aluminum based iron, vanadium and silicon containing ribbon fabricated by the present invention;

#### DESCRIPTION OF THE PREFERRED EMBODIMENTS

The aluminum base, rapidly solidified alloy appointed for use in the process of the present invention has a composition consisting essentially of the formula  $Al_{ba}Fe_aSi_bX_c$  wherein X is at least one element selected from the group consisting of Mn, V, Cr, Mo, W, Nb, Ta, "a" ranges from 1.5-8.5 at %, "b" ranges from 0.25-5.5 at %, "c" ranges from 0.05-4.25 at % and the balance is aluminum plus incidental impurities, with the proviso that the ratio  $[Fe+X]:Si$  ranges from about 2.0:1 to 5.0:1. Examples of the alloy include aluminum-iron-vanadium-silicon compositions wherein the iron ranges from about 1.5-8.5 at %, vanadium ranges from about 0.25-4.25 at %, and silicon ranges from about 0.5-5.5 at %.

Another aluminum base, rapidly solidified alloy suitable for use in the process of the invention has a composition consisting essentially of the formula  $Al_{ba}Fe_aSi_bX_c$  wherein X is at least one element selected from the group consisting of Mn, V, Cr, Mo, W, Nb, Ta, "a" ranges from 1.5-7.5 at %, "b" ranges from 0.75-9.5 at %, "c" ranges from 0.25-4.5 at % and the balance is aluminum plus incidental impurities, with the proviso that the ratio  $[Fe+X]:Si$  ranges from about 2.0:1 to 1.0:1.

Still another aluminum base, rapidly solidified alloy suitable for use in the process of the invention has a composition consisting essentially of the formula  $Al_{ba}Fe_aX_c$  wherein X is at least one element selected from

the group consisting of Mn, V, Cr, Mo, W, Nb, Ta, Ce, Ni, Zr, Hf, Ti, Sc, "a" ranges from 1.5-8.5 at %, "b" ranges from 0.25-7.0 at %, and the balance is aluminum plus incidental impurities.

Still another aluminum base, rapidly solidified alloy that is suitable for use in the process of the invention has a composition range consisting essentially of about 2-15 at % from the group consisting of zirconium, hafnium, titanium, vanadium, niobium, tantalum, erbium, about 10 0-5 at % calcium, about 0-5 at % germanium, about 0-2 at % boron, the balance being aluminum plus incidental impurities.

A low density aluminum-lithium base, rapidly solidified alloy suitable for use in the present process has a composition consisting essentially of the formula  $Al_{ba}Zr_aLi_bMg_cT_d$ , wherein T is at least one element selected from the group consisting of Cu, Si, Sc, Ti, B, Hf, Cr, Mn, Fe, Co and Ni, "a" ranges from 0.05-0.75 at %, "b" ranges from 9.0-17.75 at %, "c" ranges from 0.45-8.5 at % and "d" ranges from about 0.05-13 at %, the balance being aluminum plus incidental impurities.

Those skilled in the art will also appreciate that other dispersion strengthened, rapidly solidified alloys may be appointed for use in the process of the present invention.

The metal alloy quenching techniques used to fabricate these alloys generally comprise the step of cooling a melt of the desired composition at a rate of at least about  $10^5$  C./sec. Generally, a particular composition is selected, powders or granules of the requisite elements in the desired portions are melted and homogenized, and the molten alloy is rapidly quenched on a chill surface, such as a rapidly moving metal substrate, an impinging gas or liquid.

When processed by these rapid solidification methods the aluminum alloy is manifest as a ribbon, powder or splat of substantially uniform microstructure and chemical composition. The substantially uniformly structured ribbon, powder or splat may then be pulverized to a particulate for plasma spraying

For the purposes of this specification and claims the term fiber means a ceramic material continuous in length and not of a prescribed diameter or chemical composition. Moreover, the term reinforcement of the composite shall mean (1) an essentially nonmalleable character, (2) a scratch hardness in excess of 8 on the Ridgway's Extension of the MOHS' Scale of Hardness and (3) an elastic modulus greater than 200 GPa. However, for the aluminum matrices of this invention somewhat softer reinforcing fibers such as graphite fibers may be useful. Reinforcing fibers useful in the process of this invention include mono- and multi-filaments of silicon carbide, aluminum oxide including single crystal sapphire and/or aluminum hydroxide (including additions thereof due to its formation on the surface of the aluminum matrix material), zirconia, garnet, cerium oxide, yttria, aluminum silicate, including those silicates modified with fluoride and hydroxide ions, silicon nitride, boron nitride, boron carbide, simple mixed carbides, borides carbo-borides and carbonitrides of tantalum, tungsten, zirconium, hafnium and titanium, and any of the aforementioned fibers impregnated or encompassed with a metal such as aluminum, titanium, copper, nickel, iron or magnesium. In particular, because the present invention is concerned with aluminum based composites that possess a relatively low density and high modulus, silicon carbide and aluminum oxide are desirable as the reinforcing phase. However, de-

pending on the rapidly solidified alloy other fiber reinforcements may prove to form superior matrix/reinforcement bonds. Also, the present specification is not limited to single types of reinforcement or single phase matrix alloys.

In the process of the present invention fibers are initially placed directly on a mandrel or on a suitable substrate such as a rolled foil or planar flow cast ribbon in an amount ranging from about 0.1 to 75 percent by volume of the sprayed monotape. The mandrel may be 10 water or gas cooled, or may be heated directly or indirectly during the processing. The optimum mandrel temperature is dependent on the rapidly solidified alloy and the dispersed phases which must be formed during solidification. The rapidly solidified alloy in the form of 15 powder that can range in size from 0.64 cm in diameter down to less than 0.0025 cm in diameter may then be plasma sprayed onto the fiber-wrapped mandrel. The plasma spraying process comprises the steps of (i) ionizing an inert gas to generate a plasma; (ii) injecting said 20 powder into said plasma; (iii) controlling the residence time of said powder within said plasma to cause said powder to reach a molten state; and (iv) directing said molten powder into said substrate ionized gas plasma is 25 created for example by either a direct current (d.c.) induction coupled or radio frequency power source. Direct current plasma spraying may be performed using a 20 to 40 kW power source and more preferably between 25 to 40 kW of power. Powder flow rate into 30 the ionized plasma is dependent on the velocity of the gas exiting the nozzle of the d.c. plasma spraying unit, for if the powder is introduced into the plasma at too slow of a flow rate it will be blown back and will not enter the plasma, and if the powder is introduced at too rapid a rate, the powder will only partially melt before 35 it impinges on the substrate. Induction coupled plasma spraying may be performed using a 140 to 200 kW power level and more preferably between 150 to 170 kW of power. Powder flow rates into the ionized plasma gas are dependent only on the liquidus temperature of the alloy and the temperature of the plasma. The major advantage of induction coupled plasma spraying compared to d.c. plasma spraying is that the powder 40 residence time in the plasma is estimated to be approximately 70 times greater; thus, larger powder particles can be injected into the plasma and complete melting will occur. The term "optimum flow rate" in the context of the Present specification and claims means introducing powder into the plasma at a rate such that the powder is not rejected by the plasma and/or the powder is completely melted prior to it impinging and solidifying on the substrate. The term "optimum vacuum level" in the context of the present specification and 45 claims means regulating the vacuum level in the respective plasma spraying chambers such that the length of the plasma prevents the molten powder droplets from solidifying prior to them striking the substrate, and that the length of the plasma does not itself impinge upon the substrate and result in excessive heating of the substrate which in turn will affect the solidification rate of the deposited molten droplets or the degradation of the 50 deposited layer of powder.

Plasma spraying may be performed for varying lengths of time depending on the thickness of the sprayed preform or monotape required. In this manner there is provided a strong bond between the deposited matrix material and the surface of the reinforcing fibers. Moreover, the attractive microstructure and mechan- 55

ical and physical properties of the rapidly solidified powder are retained. This process may be repeated such that subsequent spraying is done on fibers placed on top of the sprayed monotapes, and multi-layered preforms 5 may be fabricated.

The fabricated fiber reinforced preforms may be bonded together using suitable bonding techniques such as a diffusion bonding, roll bonding and/or hot isostatic pressing, to form an engineering shape which is a substantially void-free mass. Bonding may be performed at temperatures which range from 400° C. to 575° C. and more preferably in the range from 475° C. to 530° C., under applied pressures which range from 7 MPa to 150 MPa and more preferably in the range from 34 MPa to 100 MPa. The applied pressure is dependent on the bonding temperature and optimally will be sufficient to provide a mechanical and chemical bond between preforms, yet will not break or damage the fibers present in the preform. In the case of diffusion bonding or hot isostatic pressing, vacuums greater than 100 microns are preferable. Bonding may be assisted by placing foils or powders composed of commercially pure aluminum or of a suitable alloy which is relatively soft at the bonding temperatures and allows fast diffusion of alloy constituents across the foil/preform boundaries. Moreover, fiber reinforced preforms may be oriented above one another such that the fiber reinforcement may be unidirectional, bi-directional or multi-directional. The number of laminations is dependent on the required size and thickness of the desired engineering shape. This shape may be subsequently worked to increase its density and provide engineering shapes such as sheets and plates suitable for use in aerospace, automotive and miscellaneous components.

#### EXAMPLE I

Rapidly solidified, planar flow cast ribbon of the composition aluminum balance, 4.06 at % iron, 0.70 at % vanadium, 1.51 at % silicon (hereinafter designated alloy A) was wrapped on about a 30 cm diameter steel mandrel. British Petroleum Sigma monofilament SiC fiber (hereinafter designated BP fiber) was then wrapped on top of the planar flow cast substrate. The BP fiber has an average diameter of about 104 micrometers and was wrapped in a helical configuration with about a 300 micrometer spacing. -80 mesh (U.S. standard sieve size) alloy A powder was then plasma sprayed onto the BP fiber wrapped mandrels for approximately 8 min. Plasma spraying was performed at 165 kW to deposit the required layer of rapidly solidified alloy A. FIG. 1 is a light photomicrograph of fiber reinforced plasma sprayed monotapes composed of rapidly solidified aluminum base alloy A deposited on BP placed upon planar flow cast aluminum based alloy A ribbon fabricated by the present invention. Minor amounts of porosity may be observed, however, discrete primary intermetallic compound particles are not seen in the matrix alloy A microstructure indicating that solidification of the plasma sprayed powders occurs at a rate rapid enough to suppress the formation of coarse primary dispersoid particles.

#### EXAMPLE II

Rapidly solidified, planar flow cast ribbon of the composition aluminum balance, 4.06 at % iron, 0.70 at % vanadium, 1.51 at % silicon (hereinafter designated alloy A) was wrapped on about a 30 cm diameter steel mandrel. Nicalon multifilament SiC fiber impregnated

with aluminum (hereinafter designated Nicalon fiber) was then wrapped on top of the planar flow cast substrate. The Nicalon fiber has an average diameter of about 500 micrometers and was wrapped with about a 1500 micrometer spacing -80 mesh (U.S. standard sieve size) alloy A powder was then plasma sprayed onto the Nicalon fiber wrapped mandrels for approximately 60 min. Plasma spraying was performed at 165 kW to deposit the required layer of rapidly solidified alloy A. FIG. 2 is a light photomicrograph of fiber reinforced plasma sprayed monotapes composed of rapidly solidified aluminum base alloy A deposited on Nicalon fibers, placed upon planar flow cast aluminum based alloy A ribbon fabricated by the present invention. Minor amounts of porosity may be observed, however, discrete primary intermetallic compound particles are not seen in the matrix alloy A microstructure indicating that solidification of the plasma sprayed powders occurs at a rate rapid enough to suppress the formation of coarse primary dispersoid particles.

### EXAMPLE III

Transmission electron microscopy (TEM) was performed on plasma sprayed deposited layers composed of alloy A to further examine the microstructure of the deposited layer. Samples were prepared by mechanically grinding off the planar flow cast alloy A substrate ribbon and thinning the sample to approximately 25 microns in thickness. TEM foils were prepared by conventional electro-polishing techniques in an electrolyte consisting of 80 percent by volume methanol and 20 percent by volume nitric acid. Polished TEM foils were examined in a philips EM 400T electron microscope. Transmission electron photomicrographs of a plasma sprayed deposited layer composed of rapidly solidified aluminum based iron, vanadium and silicon containing alloy is shown in FIG. 3.

### EXAMPLE IV

Plasma sprayed monotapes of BP fiber reinforced composites were diffusion bonded for preliminary mechanical property screening. Two layers of rapidly solidified, planar flow cast aluminum based 2.37 at % iron, 0.27 at % vanadium and 1.05 at % silicon containing alloy ribbon, approximately five centimeters by ten centimeters in dimension, were placed in between six layers of BP fiber reinforced plasma sprayed monotapes of approximately the same size as fabricated by the conditions prescribed to in Example I. Diffusion bonding was performed for a period of 1 hr. in a 445 kN vacuum hot press, at a temperature of approximately 500° C., under a pressure of approximately 50 MN/m<sup>2</sup>, and in a vacuum less than 10 microns of mercury. Photomicrographs of diffusion bonded layers of plasma sprayed monotapes composed of rapidly solidified aluminum base alloy A deposited on BP fiber placed upon planar flow cast aluminum base alloy A containing ribbon fabricated by the present invention is shown in FIG. 4.

### EXAMPLE V

Plasma sprayed monotapes of Nicalon fiber reinforced composites were diffusion bonded for preliminary mechanical Property screening. Six layers of rapidly solidified, planar flow cast aluminum based 2.37 at % iron, 0.27 at % vanadium and 1.05 at % silicon containing alloy ribbon, approximately five centimeters by ten centimeters in dimension, were placed in between

two layers of Nicalon fiber reinforced plasma sprayed monotapes of approximately the same size as fabricated by the conditions prescribed to in Example II. Diffusion bonding was performed for a period of 1 hr. in a 445 kN vacuum hot press, at a temperature of approximately 500° C., under a pressure of approximately 50 MN/m<sup>2</sup>, and in a vacuum less than 10 microns of mercury. Photomicrographs of diffusion bonded layers of plasma sprayed monotapes composed of rapidly solidified aluminum base alloy A deposited on Nicalon fiber placed upon planar flow cast aluminum base alloy A containing ribbon fabricated by the present invention is shown in FIG. 5.

### EXAMPLE VI

Small dog bone tensile specimens of plasma sprayed and diffusion bonded samples of BP and Nicalon fiber reinforced alloy A composites were mechanically tested to determine their ambient temperature and 482° C. fracture strength (F.S.). Tests were performed on an Instron Model 1125 tensile machine. Static Young's modulus (E), a measure of the material stiffness, was also tested using a clip on strain gauge during tensile testing at ambient temperature. Ambient and 482° C. fracture strength and ambient temperature Young's modulus for the plasma sprayed and diffusion bonded samples of BP and Nicalon fiber reinforced alloy A composites are listed in Table I.

TABLE I

| Cont. Fiber Reinforced Composite Sample Comp. | Test Temp. (°C.) | F.S. (MN/m <sup>2</sup> ) | E* (GN/m <sup>2</sup> ) |
|-----------------------------------------------|------------------|---------------------------|-------------------------|
| Alloy A/BP Fiber                              | 25               | 258                       | 105                     |
| Alloy A/BP Fiber                              | 482              | 61                        | NM                      |
| Alloy A/Nicalon Fiber                         | 25               | 114                       | 57                      |
| Alloy A/Nicalon Fiber                         | 482              | 101                       | NM                      |

\*NM refers to not measured.

Having thus described the invention in rather full detail, it will be understood that such detail need not be strictly adhered to by that further changes and modifications may suggest themselves to one skilled in the art, all falling within the scope of the invention as defined by the subjoined claims.

We claim:

1. A process for producing a rapidly solidified aluminum base metal matrix composite, comprising the steps of:
  - (a) forming a rapidly solidified aluminum base alloy into a powder;
  - (b) plasma spraying said powder onto at least one substrate having thereon a fiber reinforcing material to form a plurality of preforms wherein each of said preforms has a layer of said alloy deposited thereon and said fiber reinforcing material is present in an amount ranging from about 0.1 to 75 percent by volume thereof; and
  - (c) bonding said preforms to form an engineering shape.
2. A process as recited in claim 1, wherein said rapidly solidified alloy has a substantially uniform structure.
3. A Process as recited in claim 2, wherein said rapidly solidified aluminum base alloy is prepared by a process comprising the steps of forming a melt of the

aluminum based alloy and quenching the melt on a moving chill surface at a rate of at least 105° C./sec.

4. A process as recited in claim 1, wherein said alloy layer is strongly bonded to said fiber reinforcing material.

5. A process as recited by claim 1, wherein in sequence, prior to step (c), additional fiber reinforcing material is applied to each of said preforms and said powder is plasma sprayed thereon to modify said preforms prior to bonding.

6. A process as recited by claim 5, wherein said sequence is repeated a plurality of times.

7. A process as recited by claim 6, wherein said sequence is repeated from 2 to 10 times.

8. A process as recited by claim 5, wherein said modified preforms are bonded to form said engineering shape.

9. A process as recited by claim 5, wherein at least one of said modified preforms is bonded to at least one of said preforms to form said engineering shape.

10. A process as recited in claim 1, wherein said bonding step is at least one member selected from the group consisting of diffusion bonding, roll bonding and hot isostatic pressing.

11. A process as recited in claim 3, wherein said rapidly solidified aluminum based alloy has a composition consisting essentially of the formula  $Al_{ba}Fe_aSi_bX_c$  wherein X is at least one element selected from the group consisting of Mn, V, Cr, Mo, W, Nb, Ta, "a" ranges from 1.5 to 8.5 at %, "b" ranges from 0.25 to 5.5 at %, "c" ranges from 0.05 to 4.25 at % and the balance is aluminum plus incidental impurities, with the proviso that the ratio [Fe+X]:Si ranges from about 2.0:1 to 5.0:1.

12. A process as recited in claim 11, wherein said rapidly solidified aluminum based alloy is selected from the group consisting of the elements Al-Fe-V-Si, wherein the iron ranges from about 1.5-8.5 at %, vanadium ranges from about 0.25-4.25 at %, and silicon ranges from about 0.5-5.5 at %.

13. A process as recited in claim 3, wherein said rapidly solidified aluminum based alloy has a composition consisting essentially of the formula  $Al_{ba}Fe_aSi_bX_c$  wherein X is at least one element selected from the group consisting of Mn, V, Cr, Mo, W, Nb, Ta, "a" ranges from about 1.5-7.5 at %, "b" ranges from about 0.75-9.0 at %, "c" ranges from 0.25-4.5 at % and the balance is aluminum plus incidental impurities, with the proviso that the ratio [Fe+X]:Si ranges from about 2.0:1 to 1.0:1.

14. A process as recited in claim 3, wherein said rapidly solidified aluminum based alloy has a composition consisting essentially of the formula  $Al_{ba}Fe_aSi_bX_c$  wherein X is at least one element selected from the group consisting of Mn, V, Cr, Mo, W, Nb, Ta, Ce, Ni, Zr, Hf, Ti, Sc, "a" ranges from about 1.5-8.5 at %, "b" ranges from about 0.25-7.0 at %, and the balance is aluminum plus incidental impurities.

15. A process as recited in claim 3, wherein said rapidly solidified aluminum based alloy has a composition consisting essentially of about 2-15 at % from a group consisting of zirconium, hafnium, titanium, vanadium, niobium, tantalum, erbium, about 0-5 at % calcium, about 0-5 at % germanium, about 0-2 at % boron, the balance being aluminum plus incidental impurities.

16. A process as recited in claim 3, wherein said rapidly solidified aluminum based alloy has a composition

10 consisting essentially of the formula  $Al_{ba}Zr_aLi_bMg_cT_d$ , wherein T is at least one element selected from the group consisting of Cu, Si, Sc, Ti, B, Hf, Cr, Mn, Fe, Co and Ni, "a" ranges from about 0.05-0.75 at %, "b" ranges from about 9.0-17.75 at %, "c" ranges from about 0.45-8.5 at % and "d" ranges from about 0.05-13 at %, the balance being aluminum plus incidental impurities.

17. A process as recited in claim 1, wherein said fiber reinforcing material comprises at least one member selected from the group consisting of carbides, borides, nitrides and oxides.

18. A process as recited in claim 17, wherein said fibers are selected from the group consisting of silicon carbide and aluminum oxide.

25 19. A process as recited in claim 1, wherein said plasma spraying step comprises the steps of (i) ionizing an inert gas to generate a plasma; (ii) injecting said powder into said plasma; (iii) controlling the residence time of said powder within said plasma to cause said powder to reach a molten state; and (iv) directing said molten powder onto said substrate.

20. A process as recited in claim 19, wherein said powder has a particle size less than -40 mesh (U.S. standard sieve size).

35 21. A process as recited in claim 19, wherein said gas is ionized using a direct current, an induction coupled or radio frequency power source.

22. A process as recited in claim 10, wherein said bonding step is carried out at a temperature ranging from 400° C. to 575° C., under applied pressure ranging from 7 MPa to 150 MPa.

23. A process as recited in claim 22, wherein said bonding step is carried out under applied pressure ranging from 34 MPa to 100 MPa.

24. A process as recited in claim 1, wherein aluminum foil is placed between preforms prior to bonding.

25. A process as recited in claim 1, wherein aluminum powder is placed between preforms prior to bonding.

26. A process as recited by claim 21, wherein said power source is a direct current power source having a power level ranging from 20 to 40 kW.

27. A process as recited by claim 26, wherein said power level ranges from 25 to 35 kW.

55 28. A process as recited by claim 21, wherein said power source is an induction coupled power source having a power level ranging from 140 to 200 kW.

29. A process as recited by claim 28, wherein said power level ranges from 150 to 170 kW.

\* \* \* \* \*